

Aug. 30, 1949.

C. B. JACKSON ET AL

2,480,655

PROCESS FOR THE PRODUCTION OF ALKALI METAL

Filed Sept. 13, 1946



INVENTORS.

CAREY B. JACKSON, and  
ROBERT C. WERNER.

WITNESSES.

E. J. Maloney  
Julian B. Flick

By Brown, Critchlow, Flick, Rancham.

ATTORNEYS.

## UNITED STATES PATENT OFFICE

2,480,655

PROCESS FOR THE PRODUCTION OF  
ALKALI METAL

Carey B. Jackson, Forest Hills, and Robert C. Werner, Evans City, Pa., assignors to Mine Safety Appliances Company, Pittsburgh, Pa., a corporation of Pennsylvania

Application September 13, 1946, Serial No. 696,918

6 Claims. (Cl. 75—66)

1

This invention relates to the production of potassium as well as sodium-potassium alloys.

It has been proposed heretofore to produce sodium-potassium alloys by reacting a potassium compound, such as the hydroxide (KOH), the carbonate (K<sub>2</sub>CO<sub>3</sub>), or the chloride (KCl), with elemental sodium to produce a sodium-potassium alloy and a compound of sodium and the anion of the potassium compound used. That may be accomplished either by a batch process or by a continuous process in which the potassium compound is introduced continuously into an intermediate point of an appropriate column and sodium vapor is introduced at a point below the entry of the potassium compound. Whether practiced by the batch or the continuous procedure, the reaction conditions according to prior proposals and practice have been such that although the sodium-potassium alloy is produced satisfactorily, the procedure has not been economical because for desirable operating conditions an excess of the potassium compound, such as potassium chloride, over that theoretically necessary has been used with the result that the slag has consisted for the greater part of potassium chloride. That has been undesirable because the slag has little or no utility, and its major content of potassium chloride, which is relatively expensive, thus represents a loss; or viewed otherwise it is a major item of the cost burden of the alloy.

It has been proposed also to operate the foregoing continuous procedure in such manner as to fractionate the alloy produced, whereby pure, or substantially pure, potassium is recovered, as is advantageous for some purposes. The foregoing disadvantage has, however, equally attended such a fractionation procedure.

The primary object of the present invention is to provide a continuous process of the foregoing type that results in a slag of very low content of potassium compound and is thus substantially more economical than prior practices, and which is readily performed and does not objectionably alter or complicate the known procedures and apparatus therefor.

Other objects will be understood from the following specification.

The accompanying drawing is a flow sheet illustrative of our new method, part being broken away for clarity of illustration.

In accordance with the present invention a potassium compound reducible by sodium (Na), preferably the chloride (KCl), is heated to melt it and bring the melt to a temperature somewhat

above the melting point, and it is then fed into an intermediate point of a column, or tower, provided with appropriate packing. Sodium is vaporized and fed into the column at a point below the point of entry of the potassium compound, suitably substantially at the bottom of the column. As the molten potassium compound flows downwardly through the column it will react with the upwardly rising sodium vapor and thereby form a mixture of vapors of sodium and potassium that may be withdrawn from the upper end of the column and condensed to obtain sodium-potassium alloy, or, if preferred, the column may be operated in such manner as to effect fractionation of the alloy to recover substantially pure potassium. The slag that is formed as a result of the reaction between the potassium compound and sodium flows to the bottom of the column and is withdrawn.

20 We have discovered, and it is upon this that our invention is in large part predicated, that substantial economy with no interference in operation or with recovery of the desired alkali metal or alkali metal alloy, is to be had by passing the slag from the bottom of the column to a receiver, or re-boiler, where it is held while subjecting it to heat to drive off the sodium that the slag normally carries with it. The sodium recovered in this way is then disposed of appropriately, most suitably by returning it to the column. In this way we effect recovery of sodium that would normally be lost in the slag, and we are enabled to operate the column so that the slag as finally discharged is composed predominantly of sodium compound. This is in striking comparison with prior practice in which, to repeat, the slag was composed predominantly of potassium compound.

40 In the preferred practice of the present invention the sodium that is to be supplied to the column is likewise introduced into the re-boiler in an amount such as to form a layer overlying the slag, and the re-boiler is heated to such a temperature as to vaporize the sodium, which is then passed to the column. In this way we avoid separate heating of a source of sodium to supply vapor to the column, and at the same time the supernatant sodium layer is present to receive the sodium recovered from the slag.

45 Having reference now to the drawing, which illustrates the preferred embodiment of the invention with reference to the use of potassium chloride, molten potassium chloride, suitably at a temperature of about 1540° F., is fed to a column 50 | provided with suitable packing material, such

as stainless steel rings 2. Sodium vapor is introduced in the bottom of the column and rises upwardly therein countercurrent to the downwardly flowing molten potassium chloride. The two react to form elemental potassium and sodium chloride. The column is heated, as indicated in the drawings, to a temperature that is dependent upon the product to be recovered. Thus, if a sodium-potassium alloy is desired the column is heated so that its contents will be at a temperature somewhat above the boiling point of sodium, say to about 1620° F., whereby both sodium and potassium are vaporized and rise to the top of the column from which the mixed vapors may be withdrawn and condensed.

The salt slag that is formed flows downwardly to the bottom of the tower. In accordance with the present invention this slag is withdrawn and passed to a suitable closed receiver 3 of such size that the slag is retained for a substantial period of time before being discharged. Receiver 3 is heated to a temperature at least sufficient to maintain the slag molten and boil off the sodium that the slag carries with it, that is, to at least about 1620° F. From receiver 3 the slag is passed, preferably, to a trap 4 which is likewise heated for the purpose of driving off any traces of residual sodium that may remain in it. The sodium-free slag is then discharged from the trap 4, for instance into receivers in which it is allowed to solidify for disposal.

Preferably also, the sodium supplied to column 1 is introduced into receiver 3 to form a layer of substantial thickness that overlies the slag that is held in the receiver. Inasmuch as the slag is at a temperature above the boiling point of sodium, the metal is vaporized and fed to the column, as shown.

Desirably, an inert gas, such as nitrogen, is supplied to the system, as indicated in the drawing, to keep it under a pressure slightly in excess of atmospheric.

A further and important factor resides in our discovery that the rate of addition of the reducible potassium compound, e. g., KCl, constitutes an important factor. We believe now that the exchange reaction, between sodium vapor and the potassium compound, occurs over a relatively narrow zone adjacent the point of entry of the potassium compound. If the temperature immediately below that point be determined in relation to the slag composition it is found that better, i. e., more complete, reduction is obtained with increasing temperature. Based upon this we have found that the best results are to be had by controlling the rate of addition of the potassium compound so that a high concentration of sodium vapor will be present in the reaction zone, which is confined thereby to a small zone toward the mid-length of the column. For example, when KCl is used it enters the column at about 1550° F., and in accordance with this feature of our invention it is fed at a rate such that the temperature midway of the column is maintained between about 1575° and 1585° F., for optimum operation. If the rate of feed be increased, the mid-column temperature will fall to about 1550° F., and a high yield based on the exchange reaction will not be obtained. This is not due to change in equilibrium with temperature but rather is due to a lowered relative concentration of sodium vapor. Hence we prefer to feed the potassium compound at a rate such that there is a high concentration of sodium vapor with the reaction occurring over a narrow zone.

We find that in this way we can produce more economically a sodium-potassium alloy at least comparable in all respects to that produced in accordance with prior proposals and at the same time a slag that is both essentially free from sodium and which also consists predominantly of sodium chloride (NaCl). For example, in continuous operation the slag discharged from trap 4 consists of about 90 per cent, and there may be as much as 95 per cent, of sodium chloride, with the remainder potassium chloride. This is in direct contrast with previous procedures in which the slag produced commonly contains about 75 per cent of potassium chloride and 25 per cent of sodium chloride.

Although the invention has been described in detail with reference to the production of sodium-potassium alloy, it will be understood that pure, or substantially pure, potassium can be recovered instead of the alloy by appropriate operation of the column. Thus, pure potassium boils at atmospheric pressure at about 1420° F., and by appropriate control of the temperature gradient within the column, pure potassium may be withdrawn from the top.

We prefer to operate our process substantially at atmospheric pressure because although operation under vacuum would permit the use of lower temperatures, any advantage gained thereby would be more than offset by the added cost of apparatus strong enough to withstand the vacuum coupled with the ever present danger of collapse of some part of the apparatus, or of leakage of moisture into the system with disastrous results. Moreover, the melting point of potassium chloride is approximately 1420° F. and consequently if the pressure in the system is lowered to any extent, as would be necessary to gain advantage from operation under reduced pressure, or vacuum, the sodium vapor from the receiver, or reboiler, 3 would not be hot enough to keep the potassium chloride in a liquid state, which is essential.

According to the provisions of the patent statutes, we have explained the principle and mode of operation of our invention and have illustrated and described what we now consider to represent its best embodiment. However, we desire to have it understood that, within the scope of the appended claims, the invention may be practiced otherwise than as specifically illustrated and described.

We claim:

1. That method which comprises the steps of continuously passing a molten potassium compound reducible by sodium to a reaction column operated under substantially atmospheric pressure, continuously passing sodium vapor into said column at a point below the entry of said potassium compound, and thereby forming a sodium-potassium alloy and a slag composed predominantly of sodium and the anion of said potassium compound, withdrawing alkali metal comprising potassium from the upper end of said column, withdrawing said slag from the lower end of said column and passing it to a closed chamber, heating the withdrawn slag in said chamber to vaporize sodium carried by it, and returning the thus vaporized sodium to the column.

2. A method according to claim 1, said alloy being fractionated in said column above the point of entry of said potassium compound to produce substantially pure potassium, and withdrawing said potassium from the upper end of the column.

3. A process comprising the steps of passing

potassium chloride and sodium vapor continuously and counter-currently in a reaction column operated under substantially atmospheric pressure to produce sodium-potassium alloy and a slag composed predominantly of sodium chloride, 5 said sodium vapor being supplied to said column from a container in which a body of liquid sodium is heated to at least the boiling point of sodium, withdrawing said slag from said column and passing it through said container to vaporize 10 sodium carried by the slag and to effect further reaction between the sodium and residual potassium chloride in the slag and returning the thus vaporized sodium and recovered potassium to the system, and withdrawing alkali metal comprising potassium from the column.

4. That method which comprises the steps of continuously passing a molten potassium compound reducible by sodium to an intermediate point of a reaction column operated under substantially atmospheric pressure, continuously introducing sodium vapor into said column at a point below the entry of said potassium compound 20 to supply a high concentration of sodium vapor adjacent the entry of the potassium compound whereby the reaction



is driven to the right, thereby forming a sodium-potassium alloy and a slag composed predominantly of sodium and the anion of said potassium compound together with a minor amount of said potassium compound and sodium metal, withdrawing alkali metal comprising potassium from 30 the upper end of said column, withdrawing said slag from the lower end of said column and passing it to a closed chamber, heating the slag in said chamber to at least about 1620° F. to 35 vaporize sodium carried by the slag and to effect further reaction of sodium with residual potassium chloride carried in the slag, and returning the thus vaporized sodium and the recovered potassium to the column.

5. That method which comprises the steps of continuously introducing sodium vapor from a closed chamber heated to at least about 1620° F. into the lower end of a reaction column operated under substantially atmospheric pressure, continuously introducing molten potassium chloride at a temperature of about 1550° F. at an intermediate point of said column to produce and maintain adjacent thereto by reaction with said sodium vapor a temperature of about 1575° to 1585° F., thereby forming a sodium-potassium alloy and a slag of sodium chloride and not over about 10 percent of potassium chloride together with a minor amount of metallic sodium, withdrawing alkali metal comprising potassium from the upper end of said column, withdrawing said slag from the lower end of said column and passing it to said closed chamber, heating the slag in said chamber to vaporize metallic sodium and to effect reaction of residual potassium chloride carried by the slag, and returning the thus vaporized sodium and recovered potassium to the column.

6. A method according to claim 5, said alloy being fractionated in said column above the point of entry of said potassium chloride to produce substantially pure potassium, and withdrawing said potassium from the upper end of the column.

CAREY B. JACKSON.  
ROBERT C. WERNER.

#### REFERENCES CITED

The following references are of record in the file of this patent:

#### UNITED STATES PATENTS

| Number    | Name  | Date          |
|-----------|-------|---------------|
| 1,872,611 | Thurm | Aug. 16, 1932 |

#### FOREIGN PATENTS

| Number  | Country     | Date          |
|---------|-------------|---------------|
| 134,680 | Switzerland | Oct. 16, 1929 |